

Patented Feb. 18, 1947

2,416,021

## UNITED STATES PATENT OFFICE

2,416,021

LIGHT SENSITIVE DIAZOTYPE COM-  
POSITIONS AND PROCESSAndré Schoen, Easton, Pa., assignor to General  
Aniline & Film Corporation, New York, N. Y.,  
a corporation of DelawareNo Drawing. Application December 29, 1944,  
Serial No. 570,471

17 Claims. (Cl. 95—6)

1

The present invention relates to light sensitive photographic printing material, compositions and to the process of preparing prints therefrom.

It is an object of the invention to prepare photographic printing materials in which the color may be developed by a suitable after-treatment.

Another object of the invention is the production of photographic coating material of good stability in the dark and capable of being developed by metal salts or diazo compounds.

A further object is the provision of photographic material capable of development by diazo compounds and which are of particular value in producing dark shades of high visual density.

Another object is the provision of photographic material and the process for preparing negative prints from a pattern, or image to be reproduced, in which the image is developable by metal salts or diazo compounds.

The present invention is based upon the discovery that the arylsulfonyl compounds of aminonaphthol sulfonic acids, upon exposure to light acquire the ability to reduce metallic salts or to couple with diazo compounds. In utilizing this discovery in the practice of my invention, I coat a suitable base, carrier or support with an arylsulfonyl compound of an aminonaphthol sulfonic acid, and expose the coated carrier to light under a suitable pattern, design or picture to be reproduced, whereby the compound in those areas exposed to light is decomposed. The image in the light exposed areas then is subjected to a suitable treatment, for example, with metal salts or a suitable diazo compound, the latter treatment preferably being carried out in neutral or slightly alkaline solution, to develop a colored negative. The colors developed generally range from red through blue to black, depending on the particular aminonaphthol sulfonic acid employed and on the metal salt or diazo compound with which it is reacted. The term negative as herein employed is used relatively to the pattern or print which it is desired to reproduce, regardless of whether that pattern or print is itself a positive or a negative.

Where it is desired to employ diazo compounds to develop the color, I employ the arylsulfonyl compounds of those aminonaphthol sulfonic acids which in the free state are capable of coupling with diazo compounds. The arylsulfonyl compounds of such aminonaphthol sulfonic acids generally employed in the diazotype process, couple with diazo compounds with greater diffi-

culty than do the corresponding light decomposition products.

The non-coupling light decomposable compounds employed in the present invention are aminonaphthol sulfonic acids having the hydroxy group esterified by an arylsulfonyl group and the amino group acylated by an arylsulfonyl group, so that they may be considered as arylsulfonyl esters of aminonaphthol sulfonic acids of the probable formula:



15 wherein  $\text{ArSO}_2$  represents the residue of an arylsulfonyl group and  $n$  is a whole number of greater than zero. This formula is not intended as limiting or defining the orientation in the naphthalene nucleus of the various substituents. The

20 action of light is believed to cause hydrolysis of the ester, and in some cases also hydrolysis of the amide, resulting in the restoration of the coupling capacity of the aminonaphthol sulfonic acid.

25 In those cases where the action of light serves to hydrolyze both the ester group and the amide group, the image may be developed by treatment with a reducible metal salt to develop the color, 30 with or without a subsequent fixing treatment. In those cases where the action of light hydrolyzes the ester and not the amide, the image is developed by treatment with a diazo compound. Where it is desired to develop the image by treatment with a diazo compound, it will, of course, 35 be understood that only those aminonaphthol sulfonic acids which in the free state are capable of coupling with diazo compounds are suitable.

40 Examples of the aminonaphthol sulfonic acids which in the form of the arylsulfonyl compounds are suitable for practicing the present invention are the metathetical 1,2-aminonaphthol sulfonic acids, and 2,1-aminonaphthol sulfonic acids, such as 1-amino-2-naphthol-4-sulfonic acid, the 1-amino-8-naphthol sulfonic acids, such as 1-amino-8-naphthol-3,6-disulfonic acid, 1-amino-8-naphthol-2,4-disulfonic acid, 1-amino-8-naphthol-5,7-disulfonic acid, 1-amino-8-naphthol-4-sulfonic acid, the 2-amino-8-naphthol sulfonic acids, such as 2-amino-8-naphthol-6-sulfonic acid and 1-amino-5-naphthol-2,7-disulfonic acid, 45 I prefer to employ in the practice of my invention aminonaphthol sulfonic acids wherein the hydroxyl group is in an alpha position and the amino group is in a different nucleus and which

have a free position para to the hydroxyl group. In some of such compounds, it is preferable to also have an alpha position occupied, as for example, by a sulfonic group, whether this position be para to the alpha amino group or ortho to a beta amino group.

The arylsulfonyl compounds of aminonaphthol sulfonic acids employed in the present invention may be prepared in known manner, for example, by acting in the dark on an aminonaphthol with an arylsulfonyl chloride to acylate the amino group and esterify the hydroxy group. Suitable arylsulfonyl chlorides for this purpose are, for example, benzenesulfonyl chloride, toluenesulfonyl chloride, chlorotoluenesulfonylchloride, and the like. For example, there may be thus obtained the benzenesulfonyl ester of 1-benzenesulfonylamido-8-naphthol-4-sulfonic acid, or the 2-chloro-p-toluenesulfonyl ester of 1-(2'-chloro-p-toluenesulfonylamo)-8-naphthol -3,6- disulfonic acid and the like.

If desired, the coating may include a light stable diazo compound, as for example "Levamine Orange GSA" [2(3'-chlorobenzenediazaoamino) - p-sulfobenzoic acid] and after exposure to light the color may be developed by subjecting the base to coupling conditions, as for example, steam in the presence of acetic acid vapor. Or, in those cases where the light decomposition product is a free amine, by treatment with nitrous acid, the amine is diazotized and couples with itself to form a colored image.

The diazo compounds employed for treating the light exposed base may be in any suitable form, for example, in the form of the zinc chloride double salt, tin chloride double salt, cadmium chloride double salt, boron tetrafluoride double salt, the chloride, sulfate, or the like. In particular, those diazo compounds which contain one or more etherified phenolic groups are preferred. Examples of diazo compounds that may be employed are the diazo compounds of diethylaminoaniline, o-dianisidine, o-phenetidin, 4-chloro-2-anisidine, 4-benzoylamino-2,5-diethoxyaniline, 4-benzoylamino-2,5-dimethoxyaniline, or p-amino-phenylmorpholine.

The light sensitive compounds to which this invention relates may be applied in the dark in the form of their alkali metal or ammonium salts to a hydrophilic base or support of paper, gelatin coated cellulose acetate film or the like, preferably in the form of the aqueous solution, and the base so treated is then dried and is ready for use. In particular, for developing the latent image with metal salts, I prefer to employ mercury salts and salts of the metals above mercury in the electromotive series, as for example silver nitrate or ammoniacal silver nitrate. Where mercuric salts are employed, I use an after-treatment with ammonia to develop a black color in the reduced mercurous image.

The invention will be described in greater detail in connection with the following examples which are given to illustrate the invention.

#### Example 1

A solution is prepared containing 4 grams benzenesulfonyl ester of 1-benzenesulfonylamido-8-naphthol-4-sulfonic acid in 50 cc. water to which has been added about 0.5 cc. concentrated aqueous ammonia. This solution is then coated on paper in the dark in any suitable manner, and after drying is exposed to light under a negative. The exposed paper then is immersed in an aqueous solution containing about 1% zinc chloride double

salt of o-ethoxybenzenediazonium chloride which results in the development of a reddish purple positive. The print is then washed and dried.

#### Example 2

A solution is prepared containing about 5 grams of 2'-chloro-p-toluenesulfonyl ester of 1-(2'-chloro - p - toluenesulfonylamido)-8-naphthol-3,6-disulfonic acid in 50 cc. water containing about 0.5 cc. concentrated aqueous ammonia. This solution is applied on a suitable gelatin coated paper, dried, and the coated paper is exposed to light under a negative. The color is developed by treatment with a 1% solution of the diazonium chloride of 4-benzoyl amino-2,5-diethoxyaniline containing about 1% sodium acetate. There is thus produced a blue positive image.

#### Example 3

A solution is prepared containing about 3 grams benzenesulfonyl ester of 1-benzenesulfonylamido-2-naphthol-4-sulfonic acid in 5 cc. concentrated ammonia and 100 cc. water. This solution is applied on a suitable gelatin coated paper, dried, and the coated paper is exposed to light under a negative. The image may be developed by dipping the paper into a bath containing about 5 grams silver nitrate in 100 cc. water, and then heating the paper or exposing it to ammonia fumes. The excess silver nitrate may be washed away by immersion in a 2% solution of sodium thiosulfate, and the paper is then washed and dried.

I claim:

1. The process which comprises exposing to light under a pattern to be reproduced, a base carrying an arylsulfonyl ester of an arylsulfonylamidophenol sulfonic acid until decomposition thereof occurs, and developing the latent image by reaction with a member of the group consisting of salts of metals above mercury in the electromotive series and diazo compounds.
2. The process which comprises exposing to light under a pattern to be reproduced, a base carrying an arylsulfonyl ester of an arylsulfonylamidophenol disulfonic acid until decomposition thereof occurs, and coupling the decomposed product thereof with a diazo compound.
3. The process which comprises exposing to light under a pattern to be reproduced, a base carrying an arylsulfonyl ester of a 1-arylsulfonylamido-8-naphthol sulfonic acid until decomposition thereof occurs, and coupling the decomposed product thereof with a diazo compound.
4. The process which comprises exposing to light under a pattern to be reproduced, a base carrying an arylsulfonyl ester of a 1-arylsulfonylamido-8-naphthol disulfonic acid until decomposition thereof occurs, and coupling the decomposed product thereof with a diazo compound.
5. The process which comprises exposing to light under a pattern to be reproduced, a base carrying an arylsulfonyl ester of 1-arylsulfonylamido-2-naphthol sulfonic acid until decomposition thereof occurs, and developing the latent image by reaction with a member of the group consisting of salts of metals above mercury in the electromotive series and diazo compounds.
6. The process which comprises exposing to light under a pattern to be reproduced, a base carrying an arylsulfonyl ester of a 1-arylsulfonylamido-2-naphthol sulfonic acid until decomposition thereof occurs, and developing the latent

image with a salt of a metal above mercury in the electromotive series.

7. The process which comprises exposing to light under a pattern to be reproduced, a base carrying an arylsulfonyl ester of 1-arylsulfonamido-2-naphthol-4-sulfonic acid until decomposition thereof occurs, and developing the latent image by coupling the decomposed product thereof with a diazo compound.

8. The process which comprises exposing to light under a pattern to be reproduced, a base carrying an arylsulfonyl ester of 1-arylsulfonamido-8-naphthol-3,6-disulfonic acid until decomposition thereof occurs, and developing the latent image by reaction with a member of the group consisting of salts of metals above mercury in the electromotive series and diazo compounds.

9. The process which comprises exposing to light under a pattern to be reproduced, a base carrying the benzenesulfonyl ester of 1-benzene-sulfonamido-8-naphthol-4-sulfonic acid until decomposition thereof occurs, and coupling the decomposed product thereof with a diazo compound of o-phenetidine.

10. The process which comprises exposing to light under a pattern to be reproduced, a base carrying 2-chlorotoluenesulfonyl ester of 1-(2'-chloro-toluenesulfonamido)-8-naphthol-3,6-disulfonic acid until decomposition thereof occurs and coupling the decomposed product thereof with a diazo compound of 4-benzoylamino-2,5-diethoxyaniline.

11. Light sensitive material which comprises a base carrying a light sensitive arylsulfonyl ester of an arylsulfonamidonaphthol sulfonic acid.

12. Light sensitive material which comprises a base carrying a light sensitive arylsulfonyl ester of an arylsulfonamido naphthol disulfonic acid.

13. Light sensitive material which comprises a base carrying a light sensitive arylsulfonyl ester of 1-arylsulfonamido-2-naphthol disulfonic acid.

14. Light sensitive material which comprises a base carrying a light sensitive arylsulfonyl ester of a 1-arylsulfonamido-8-naphthol-4-sulfonic acid.

15. A light sensitive material comprising a base carrying an arylsulfonyl ester of 1-arylsulfonamido-8-naphthol-3,6-disulfonic acid.

16. A light sensitive material comprising a base carrying an alpha arylsulfonyl ester of an arylsulfonamido-alpha naphthol sulfonic acid having a free position para to the hydroxyl group and wherein the hydroxy and amino groups are in different nuclei.

17. A light sensitive material comprising a base carrying a light sensitive arylsulfonyl ester of an arylsulfonamido-alpha-naphthol sulfonic acid having a free position para to the hydroxyl group.

ANDRÉ SCHOEN.

#### REFERENCES CITED

The following references are of record in the file of this patent:

#### UNITED STATES PATENTS

|    | Number    | Name           | Date          |
|----|-----------|----------------|---------------|
| 25 | 1,751,318 | Gay            | Mar. 18, 1930 |
|    | 1,934,011 | Schmidt et al. | Nov. 7, 1933  |
|    | 2,034,508 | DeBoer et al.  | Mar. 17, 1936 |
| 30 | 2,095,408 | DeBoer et al.  | Oct. 12, 1937 |
|    | 2,362,598 | Vittum et al.  | Nov. 14, 1944 |
|    | 2,067,690 | Alink et al.   | Jan. 12, 1937 |
|    | 2,083,285 | Alink et al.   | June 8, 1937  |
| 35 | 2,150,834 | Holst et al.   | Mar. 14, 1939 |
|    | 2,183,447 | Dippel et al.  | Dec. 12, 1939 |
|    | 2,216,137 | Schmidt et al. | Oct. 1, 1940  |
|    | 2,311,016 | Alink et al.   | Feb. 16, 1943 |

#### FOREIGN PATENTS

|    | Number  | Country | Date         |
|----|---------|---------|--------------|
| 40 | 283,274 | British | Jan. 6, 1928 |